

May 11, 1971

SHINNOSUKE FUNAKUBO

3,578,512

METHOD OF HEAT TREATMENT OF A STEEL PRODUCT

Filed May 17, 1968

*Fig. 1*



*Fig. 2*



*Fig. 3*



*Fig. 4*



INVENTOR

SHINNOSUKE FUNAKUBO

BY *Oto John Murray*  
ATTORNEY

## 1

3,578,512

### METHOD OF HEAT TREATMENT OF A STEEL PRODUCT

Shinnosuke Funakubo, Tokyo, Japan, assignor to Funakubo Seikyo Kabushiki Kaisha, Tokyo, Japan  
Filed May 17, 1968, Ser. No. 730,120  
Claims priority, application Japan, May 25, 1967,  
42/32,789  
Int. Cl. C21d 9/32

U.S. CL. 148—147

6 Claims

### ABSTRACT OF THE DISCLOSURE

A method of heat-treating and hardening a steel product such as a toothed wheel and similar structural elements, requiring a hardness and abrasion resistance on portions of its working surfaces increased in comparison to the hardness and abrasion resistance of the remaining portions comprising the steps of providing on the surface of said product at least one groove separating the said surfaces of portions of required increased hardness from the remaining surfaces; locally heat-treating the said portions of the surfaces requiring an increased hardness as they are divided by said at least one groove and subsequently hardening by quenching the heat-treated portions leaving the remaining portions with its original hardness and abrasion resistance.

### BACKGROUND OF THE INVENTION

#### Field of the invention

The present invention relates to a method of heat treatment of a steel product, particularly working parts of machines such as a toothed wheel.

#### Description of the prior art

Most of toothed wheels and other steel working parts of machines are essentially required to be hardened extremely and locally at their working portion such as a tooth portion of a toothed wheel, and are to retain toughness at their other bottom or central portions. The conventional hardening, for satisfying the above requirement, has been conducted in the way that for example, a heated chisel is cooled locally at a predetermined hardening portion with a quenching agent, and after that, tempered at said portion with excess heat other portions remaining not cooled. The method is applicable to chisels and tools, the hardening portions of which are straight, but not to toothed wheels, the hardening portions of which extend radially. For improving the abrasion resistance on surfaces of the work portions of steel products, a flame-hardening or high-frequency hardening has been employed for casehardening around their working surfaces. This method is difficult to use in the surfaces locally and limitedly.

### SUMMARY OF THE INVENTION

An object of the present invention is, hence, to provide a method of heat treatment of a steel product, particularly a toothed wheel and other structural elements of machines, having predetermined hardening portions capable of heating and hardening locally and limitedly with other portion remained unhardened and reducing to the minimum the probability of distortion which has been encountered on heated products of the prior art.

The principle of the present invention is, therefore, to provide a method of heat treatment of a steel product, such as a toothed wheel and similar structural elements, which comprises providing one or more grooves between the portions to be hardened and other portions not to be hardened, and subjecting said firstly-mentioned portion

## 2

to a heating atmosphere. The heat applied to said firstly-mentioned portion is hindered from transmission to said secondly-mentioned portion, because of the existence of said grooves, and said secondly-mentioned portion remains unaffected by the heat treatment.

### DESCRIPTION OF THE DRAWINGS

In the accompanying drawings showing preferred embodiments of a structural element to be heated by the heating method of the present invention.

FIG. 1 shows a plan view of a toothed wheel provided with a heat transmission inhibiting groove of the present invention to be treated by a heating method of the present invention;

FIG. 2 shows a sectional view taken along the line II—II of FIG. 1;

FIG. 3 is an explanatory diagram showing a transmission of heat applied to the toothed wheel from the direction of a projected portion, to be hardened and

FIG. 4 is a partial view in perspective showing another embodiment of the toothed wheel treated by the heating method of the present invention.

### DESCRIPTION OF THE PREFERRED EMBODIMENTS

In the drawings, a toothed wheel 1 is shown having a number of teeth 2 provided with a hole 4 for a central axis. On each end surface of said toothed wheel 1, a circular groove 3 is provided around the outer periphery of the portion to be hardened and at a certain distance therefrom. When heat generated, for example by a high-frequency electromagnetic field or a flame, is applied to the tooth portion of said toothed wheel from the direction of the projected portion, said tooth portion, appreciably, is heated rapidly, but the remaining portion between the axis and the groove 3 remains not heated. A distribution of the heating temperature onto the toothed wheel is shown in FIG. 3, the diagram of which is based upon the tempering color surface as it appeared on each surface of toothed wheel.

Apparently the groove 3 serves to prevent transmission of the heat applied to the tooth portion in the direction of the centre of axis, but this premise is not clear. In heating by a high-frequency electromagnetic field, the groove 3 seems to work to cut off line of magnetic force.

If the thus heated toothed wheel is quenched, said toothed wheel is hardened only at the tooth portion, but remains unhardened at the portion nearer to the axis or the basic portion.

In another embodiment shown in FIG. 4, plural grooves 3 are provided radially inwardly of the teeth of the toothed wheel and extending in the axial direction thereof.

The deeper the groove the greater is the hindrance of heat transmission, but an excessive increase in depth of the groove would cause a concentration of stress onto the groove, leading to damage or breakdown around the grooved portion during practical application of the toothed wheel. The most efficient groove therefore has a depth which does not interfere with maintaining the basic portion confined by the groove at a temperature below the transformation point of the toothed wheel, if the temperature around the tooth portion reaches to the transformation point.

What is claimed is:

1. A method of heat treatment and hardening of a steel product, to provide it with a hardened working portion having a working surface and a remaining portion with its original hardness, such as a toothed wheel and similar structural elements which comprises the steps of:

providing at least one groove in the surface of said product, between the said working portion to be hardened and the remaining portion, which is not to be hardened;

subjecting said working surface portion to be hardened to a heating treatment and subsequently hardening said working portion by quenching

the heat applied to the said working portion is hindered by said groove from transmission to the remaining portion, and the said remaining portion is substantially unaffected by the heat treatment.

2. A method of heat treatment of a steel product as claimed in claim 1, the heat being applied to said working portion by high-frequency heating.

3. A method of heat treating a steel product as claimed in claim 1, the heat being applied at a temperature above the transformation point of said working portion.

4. A method of heat treating a steel product as claimed in claim 1, the heat being applied by a flame.

5. A method of heat treating a steel product as claimed in claim 1, said steel product comprising a gear with

wheel teeth, said groove being an annular groove provided on each face of the gear wheel radially inwardly of the teeth.

6. A method of heat treating a steel product as claimed in claim 1, said working portion of said product being a tooth of a gear, said groove being an axially extending groove provided on each side of the tooth at its base.

#### References Cited

##### UNITED STATES PATENTS

2,430,005 11/1947 Denneen et al. ----- 148—149

RICHARD O. DEAN, Primary Examiner

10 U.S. Cl. X.R.

15 148—149, 150, 151, 152